

## UNITED STATES PATENT OFFICE

WERNER STAUFFER, OF ZURICH, SWITZERLAND, ASSIGNOR TO THE FIRM AKTIEN-  
GESELLSCHAFT DER MASCHINENFABRIKEN ESCHER WYSS & CIE., OF ZURICH,  
SWITZERLAND

## PROCESS FOR HARDENING HIGH-SPEED STEEL

No Drawing. Application filed April 7, 1928, Serial No. 268,375, and in Switzerland April 23, 1927.

It is known that when so-called "high speed steel" is heated after hardening in an ordinary open forge fire or in any kind of furnace, a soft zone of greater or less thickness is produced, by decarbonization, and has to be removed by grinding it off. This phenomenon, which is the cause of severe wear in high speed steels, appears in a particularly inconvenient form in the case of shaped pieces, complicated parts, and articles which, after hardening, have to be reduced to exact dimensions by grinding and must, besides possess the highest possible degree of superficial hardness.

Hitherto the procedure in such cases has been to pack the pieces into a box, of sheet iron or a heat resisting alloy, containing wood charcoal, coke breeze or cinders (wrapping the articles in paper and then heating them in a well closed box is also a common practice in some places), the whole being then brought to hardening temperature, after which the articles are removed from the box and quenched.

This method yielded passable results provided the temperature was not raised above 1200° C. Furthermore, meticulous care had to be taken to remove the articles from the box and quench them as soon as they had reached hardening temperature. If these points were not attended to and if the temperature were increased or the time of heating prolonged the marginal zones rapidly became carbonized and melted off as the melting point of the metal was thereby reduced far below the temperature most suitable for hardening.

Under these conditions the corners and edges of the articles were inevitably damaged. Such a steel would, in the hardening shops, be described as "overcooked", and it was generally supposed that in such cases, the hardening temperature had been pushed to too high a limit. The disadvantages cannot, moreover, be prevented by heating the articles in a cinder bed. The reason is that the cinders contain a certain amount of unburnt coal so that local carbonization, at least, must still take place. If, on the other hand, the cinder bed is practically free from combustible constituents, the articles will be decarbonized and, furthermore, the cinders sinter together

at high temperatures and become caked on to the articles to be hardened.

It frequently happens that appreciable melting off is not noticed notwithstanding the fact that the outer surface is more or less heavily carbonized. In such a steel, owing to its non-homogeneous composition, severe stresses are set up during hardening and these, in subsequent working, or even during hardening may give rise to the formation of cracks and flaking. Furthermore the cutting edge does not maintain its shape but scales off easily.

In order to overcome these disadvantages as completely as possible it has thus been necessary to carry out the hardening of high speed steel with scrupulous accuracy and to observe the above mentioned points exactly.

Also, since the recent introduction of modern cobalt high speed steels requiring a hardening temperature up to 1380° C., it has been customary to treat such articles which have to be packed according to the old method. As however these steels attain their maximum efficiency only after hardening at the highest temperature, shortly below their melting point, and since such temperatures are not admissible when proceeding according to the methods hitherto known, the use of so expensive a material entailed merely a useless waste of money.

The process which forms the subject matter of the present invention avoids all these disadvantages and makes the hardening of high speed steel much more independent of the skill of the hardener. This new process consists in packing the articles to be hardened, during heating, in at least one carbide in a finely divided form. "Carbide in a finely divided form" must here be understood to mean a granular and powdered carbide.

For example, for the hardening of high speed steel a silicon carbide in a granular form can be used, whereby the temperature can be raised to 1380° C. without the piece of steel suffering damage or burning.

When working according to the now process it is possible to attain good protection from sintering without any considerable degree of carbonization taking place, as a slight-

55

60

65

70

75

80

85

90

95

100

ly reducing atmosphere is formed. Caking on of the packing material does not take place and the latter can be used over again as many times as may be desired, so that the consumption of such material is small. If the reducing action of the repeatedly used silicon carbides has fallen off too much, a small quantity of a more easily oxidizable material such as graphite powder, for example, may be added. Whereas wood charcoal and cinders are bad conductors of heat the carbides, particularly silicon carbide, conduct heat very well. Thus it follows that, in carrying out the new process, owing to the uniform and rapid heating through the vessels, a substantial saving of fuel is effected and a considerably increased output obtained. Furthermore steels hardened by the new process exhibit very favourable properties, since in the structure, owing to the short time of the heating, the transformation of small points of carbide into large complexes scarcely takes place at all.

I claim:

A process for hardening high speed steel articles, consisting in packing the articles to be hardened preliminarily to their heating, in silicon carbide in a finely divided form, and in keeping said articles packed therein during heating.

In testimony whereof I have signed my name to this specification.

WERNER STAUFFER.